

Jan. 9, 1923.

W. E. SUMNER,  
FLOOR COVERING.  
FILED MAY 12, 1922.

1,442,012.



Inventor

Warren E. Sumner,  
By Dodge and Dow,  
Attorneys

## UNITED STATES PATENT OFFICE.

WARREN E. SUMNER, OF EAST WALPOLE, MASSACHUSETTS, ASSIGNOR TO BIRD & SON, INC., A CORPORATION OF MASSACHUSETTS.

## FLOOR COVERING.

Application filed May 12, 1922. Serial No. 560,842.

*To all whom it may concern:*

Be it known that I, WARREN E. SUMNER, a citizen of the United States, residing at East Walpole, in the county of Norfolk and State of Massachusetts, have invented certain new and useful Improvements in Floor Coverings, of which the following is a specification.

This invention pertains to floor coverings and has reference more particularly to coverings of the type set forth and claimed in Letters Patent No. 1,131,317, granted to me under date of March 9th, 1915.

The object of the present invention is to produce a covering wherein the backing coating or under surfacing thereof is of a more durable character than that heretofore employed, with the result that it will not pulverize, and as a consequence does not dust off. Again, the backing composition is such that it does not tend to mask the pigment which may be employed to produce the desired color.

A section of the floor covering is illustrated in the annexed drawing, the various coatings being shown on a somewhat enlarged scale so as to clearly depict the same.

As in the structure set forth in the aforesaid patent it is designed to have the body proper produced from a waterproofed material, such, for instance, as felt, impregnated with a suitable asphalt. Such body is denoted by 1 in the drawing and has imposed thereon any suitable wear resisting surface, as, for instance, a coating 2 of paint and, if desired a printed pattern or design surface 3. The undercoating or backing denoted by 4 is composed of the following ingredients in approximately the

following proportions:

38 lbs. of Montan wax

57 " of hardened rosin-paraffin

5 " of 135° paraffin, and a suitable pigment, say 11 lbs. of red oxide ground in oil, where a red tone, for instance, is desired.

Preferably the hardened rosin paraffin is produced by heating the rosin to a high temperature and before it solidifies blending sufficient paraffin therewith in order that the mixture thereby produced may be melted over a steam bath. When so melted the remaining ingredients may be admixed therewith.

The rosin may, however, be first hardened in a kettle and the remainder of the ingredients added thereto, but the method above outlined is preferred as it permits greater convenience in blending.

Such admixture produces a waxy compound which is found distinctly advantageous over that wherein the Montan wax is predominant. As above noted the compound does not mask the pigment and, while just as adherent to the body 1, it does not pulverize and flake or dust off, this seemingly being due to the presence of the relatively large amount of paraffin in the mixture. The mixture should, of course, be applied in a heated condition to the body 1, in order that effective adhesion and bonding be effected.

What is claimed is,—

1. As a new article of manufacture, floor covering comprising a waterproofed flexible body and an undercoating containing hardened rosin and paraffin.

2. As a new article of manufacture, floor covering comprising a flexible body having an undercoating containing hardened rosin and paraffin, the rosin being present in at least half of the amount of the mixture composing the coating.

3. As a new article of manufacture, floor covering comprising a flexible body having an undercoating containing hardened rosin, paraffin, and Montan wax, the rosin and wax being present in the mixture composing the coating upwardly of at least 60%.

In testimony whereof I have signed my name to this specification.

WARREN E. SUMNER.